

Dec. 7, 1965

J. W. NIELSEN

3,221,395

METHOD OF MAKING A MICROWAVE ELEMENT

Filed May 17, 1962

Fig. 1



Fig. 2



Fig. 3

INVENTOR:  
James W. Nielsen  
By Alan C. Rose  
Attorney

## 1

3,221,395

## METHOD OF MAKING A MICROWAVE ELEMENT

James W. Nielsen, Berkeley Heights, N.J., assignor to Airtron, Inc., Morris Plains, N.J.  
Filed May 17, 1962, Ser. No. 195,625  
6 Claims. (Cl. 29—155.5)

The present invention relates to ferromagnetic materials, and more particularly to ferromagnetic materials employed in microwave devices.

In the field of microwave limiters and filters, the use of ferromagnetic materials such as ferrites has been proposed heretofore. One technical article which relates to this subject matter is entitled "Low Temperature Microwave Power Limiter," by F. J. Sansalone and E. G. Spencer, page 272 of the May 1961 issue of the I.R.E. Transactions on Microwave Theory and Techniques. In the limiters disclosed in the prior art, suitable ferromagnetic materials are employed as the coupling element between two microwave circuits to produce a form of saturation, and this nonlinear effect provides a relatively constant output for varying signal input levels.

In accordance with the teachings of Harry Suhl in "Ferromagnetic Resonance at High Signal Powers," Journal of Phys. and Chem. of Solids, vol. 1, pp. 209-227, April 1957, it is particularly important to have a relatively narrow resonance line in order to get low level limiting. Various techniques for reducing the width of the resonance line have included polishing the surface, and heat treatment. While these two techniques have been found helpful, prolonged grinding or extending heating have actually been found to produce adverse effects, in that the line width is increased rather than progressively decreased.

A principal object of the present invention is to decrease the resonance line width of ferromagnetic materials. A collateral object of the present invention is to produce an improved microwave limiter by reducing the microwave signal threshold level for the onset of nonlinearity and limiting.

In accordance with the present invention, it has been determined that the increase in line width resulting from progressive grinding is probably a result of growth induced crystal anisotropy. Thus, in the growth of crystals, certain slight changes in composition occur. As the layers are progressively ground off the outer surface of the crystal, the line width increases and decreases in a cyclic manner as slight changes in the surface composition take place. Furthermore, in accordance with the present invention, it has been determined that the increase in line width following heat treatment of certain ferromagnetic materials is due to the loss of volatile components which are present in the ferrites. Thus, heating has the desired effect of relieving strain but produces the adverse effect of changing the chemical composition through the loss of the volatile component. This adverse effect can be inhibited by providing the sphere with an excess of the volatile component in question during the heating or annealing step. Under these circumstances, the line width is reduced by strain relief and no counterbalancing increase in line width from chemical composition changes occurs.

One important limiter material is lithium ferrite. The volatile nature of the lithium has produced an undesired increase in line width upon heat treatment, as noted above. By coating with any suitable lithium-containing solution or slurry, the loss of lithium which would otherwise occur upon heating, is prevented. It is contemplated that other ferromagnetic materials containing volatile components can be handled in a similar manner to prevent changes in chemical composition.

In accordance with a feature of the invention, an ele-

## 2

ment of microwave ferromagnetic material having at least one volatile component is ground, and is subsequently heat-treated in the presence of an excess of the volatile component to relieve strain and increase the uniformity of the crystalline structure. A collateral feature involves the use of the resultant substantially isotropic and strain-free element in a microwave device, particularly for improved low-level limiting.

Through the use of the present techniques, microwave resonance line widths of less than three oersteds have been obtained, as contrasted with values of six oersteds or more, which was the lowest value that had been reported previously for spinel ferrites.

Other objects, features and advantages of the invention will become apparent upon consideration of the following detailed description when taken in combination with the accompanying drawings.

In the drawings:

FIGS. 1 and 2 are plots of the change in ferromagnetic resonance line width with grinding and heat treatment, respectively; and

FIG. 3 is a schematic showing of a microwave limiter employing a ferromagnetic coupling element treated in accordance with the principles of the present invention.

In accordance with the article by Harry Suhl cited above, the expression for the critical field for the onset of nonlinear effects is as follows:

$$h_{\text{crit}} \approx \frac{\Delta H \Delta H_k}{4\pi M_s} \quad (1)$$

where  $\Delta H$  is the line width,  $\Delta H_k$  the spin wave line width, and  $4\pi M_s$  is the saturation magnetization. Since  $h_{\text{crit}}$  should be as small as possible for limiting,  $\Delta H$  should be as small as possible.

In the course of one illustrative implementation of the principles of the present invention, lithium ferrite crystals were grown from molten lead oxide solutions which were cooled slowly from 1250° C. Chemical analyses of the crystals showed a formula of  $\text{Li}_{0.51}\text{Fe}_{2.5}\text{O}_4$ . The direct current resistivity of the crystals was about 100 ohm-centimeters. At room temperature, the saturation magnetization, designated  $4\pi M_s$ , was equal to  $3550 \pm 40$  gauss.

Rough ground spheres of the crystalline lithium ferrite had a ferromagnetic resonance line width which were more than 40 oersteds. The line width measurements were made at five kilomagcycles at room temperature, using a technique in which the sphere orients itself in an applied magnetic field, as described by R. C. LeCraw and E. G. Spencer, "Line Width Narrowing in Gallium Substituted Yttrium Iron Garnet," Bulletin of American Physical Society, p. 85, January 1960. Upon polishing the sphere with successively finer grits, the line width decreased. After four or five hours of polishing, diamond grit having an average particle size of 0.25 micron was employed. Further polishing decreased the line width to about 7.5 oersteds. With prolonged polishing, the line width rose and fell in a periodic manner as shown in FIG. 1 of the drawings.

The plot of FIG. 1 is typical of plots which were obtained by a grinding of many other lithium ferrite crystals of slightly different composition. In each case the line width varied with progressive polishing and in most instances a minimum value of about 7.5 oersteds for the line width was obtained.

Grinding with the finest aluminum oxide grit, having a chemical formula of  $\text{Al}_2\text{O}_3$  and a particle size of about 0.3 micron, appeared to increase the line width, although the periodiv change was still observed. With reference to the curve of FIG. 1, the section of the characteristic between point 12 and point 14 was ground using the diamond grit, and the section of the curve to the right of point 14 was obtained with the aluminum oxide grit.

The switch to aluminum oxide was made to improve the surface finish, as the aluminum oxide is softer and has more uniform particle size than the diamond grit.

The crystals at the first "polishing minimum" were pitted in an irregular manner. Yttrium iron garnet in the same state of polish exhibits a line width of several oersteds.

FIG. 2 illustrates the effect of heat treatment at 800° C. of a ground and polished sphere of lithium ferrite. Following about five hours of heat treatment in air, a minimum line width of about 5 oersteds was obtained. This figure was typical of the curves which were obtained for many additional spheres. In nearly every case, either in air or oxygen, the line width decreased to about the same value, regardless of the initial value. This data holds for all of the spheres which had been polished to or beyond the first "polishing minimum." The average minimum line width was about 2 oersteds less than the minimum line width obtained by polishing. The lack of difference in this minimum between samples treated in oxygen and those treated in air indicates that the decrease in line width does not depend significantly on the oxidation of divalent iron at the surface.

Treatment at 800° C. permits the mobile lithium ions to "smooth out" the slight periodic irregularities in the composition of the ferrite which are present in the form in which it is crystallized from the melt, and the heat treatment simultaneously relieves strain through annealing action. Further polishing verifies these facts, in that the resonance line width varies but slightly with additional polishing after the heat treatment. The slight further variations are attributable to variations in strain caused by the further polishing action.

The increase in resonance line width with prolonged heating at 800° C. in the absence of a coating solution is principally attributable to the vapoization of lithium. This loss is corroborated by the decrease in resonance line width which occurs with heat treatment when the spheres have been previously coated with a solution or a slurry of a lithium-containing substance.

With regard to the solutions which may be employed for treating the lithium, any suitable solution containing available lithium may be employed. A water solution of lithium carbonate has been employed successfully. Other suitable lithium salts which may be put into solution or into a slurry for application to the sphere prior to heat treatment include lithium nitrate and lithium chloride. Solvents other than water may, of course, be employed, with due care being taken in the case of inflammable solvents.

Following heat treatment in the presence of an excess of lithium, the lithium ferrite element is annealed and substantially strain-free. In addition, it has a concentration of lithium which is substantially the same at its surface as just within its surface. This substantially isotropic composition, in combination with the strain-free state of the ferrite element, are believed to account for the low resonance line width which is achieved.

FIG. 3 represents a typical limiter junction in which signals from one of the transmission lines 22 are coupled to the other transmission line 24 by the ferrite sphere 26 of improved material. The structure of FIG. 3 represents a pair of crossed coaxial waveguides having conductors 22 and 24 within the rectangular waveguide channels 28 and 30, respectively. Insulating supporting elements 32 and 34, which may, for example be made of polyfoam, hold the conductors 22 and 24, as well as the sphere 26 in their proper relative positions.

The sphere 26 must be magnetically biased with a steady magnetic field oriented perpendicular to the two transmission lines 22 and 24. This may readily be accomplished by a pair of magnets 36 and 38. The magnet structure may have a closed external loop to complete the magnetic circuit; it may also be a permanent magnet

arrangement instead of the electromagnets shown in FIG. 3.

With regard to the temperatures for heat treatment, a temperature of about 800° is preferred for lithium ferrite annealing or strain relief. However, temperatures from 720° to 900° may be used. At lower temperatures the annealing proceeds more slowly, and at higher temperatures excessive chemical changes of the ferrite may occur.

Concerning materials, the lithium ferrite advantageously has a composition near the  $Li_{0.5}Fe_{2.5}O_4$  proportions set forth hereinabove. However, limiter action may still be obtained with substantial departures from these proportions. Thus, for example, the amount of lithium in the lithium ferrite may range from that given by the formula  $Li_{0.1}Fe_{2.95}O_4$  to much greater proportions of lithium, such as  $Li_{1.5}Fe_{2.2}O_4$ , for example. Microwave materials containing other volatile components such as gallium, in addition to or instead of lithium, may also be employed. The use of an excess of the volatile component, or components, in the course of heat treatment, will avoid changing the characteristics of the material by chemical composition changes.

Another process known as "ordering" may also be used to further reduce the resonance line width to a minor extent. Ordering involves the regularity of the distribution of substituents in a crystal lattice. In the case of lithium ferrite having the formula  $(Fe)[Li_{1.5}Fe_{1.5}]O_4$ , where the parentheses indicate location in the tetrahedral sites of the spinel crystal lattice and the brackets indicate location in the octahedral sites of the spinel, the lithium atoms share the octahedral sites with the iron atoms. It had previously been determined that an arrangement wherein the lithium atoms were regularly spaced between successive sets of three iron atoms has a slightly lower resonance line width than other less ordered arrangements. This ordering occurs most rapidly at temperatures below and close to 700° C. At temperatures above 700° C., the crystal assumes a disordered state.

Accordingly, following the heat treatment at 800° C. for strain relief, a subsequent heat treatment close to 700° C. is performed for ordering.

For completeness, it is interesting to note that the frequency range for microwave materials is roughly proportional to the saturation magnetization. Thus, the useful frequency range for yttrium iron garnet, having a saturation magnetization of about 1750 gauss, is about 2,000 to 4,000 megacycles; while the useful frequency range for lithium ferrite, having a saturation magnetization of about 3,500 to 3,900 gauss, is about 5,000 to 7,000 megacycles. For this last mentioned high frequency range the present method has produced the lowest resonance line widths which have been obtained up to the present time.

It is to be understood that the above-described arrangements are illustrative of the application of the principles of the invention. Numerous other arrangements may be devised by those skilled in the art without departing from the spirit and scope of the invention. Thus, by way of example and not of limitation, certain aspects of the invention are applicable to other microwave materials which include volatile components, such as gallium doped yttrium iron garnet or lithium ferrite including some low melting point gallium material. In addition, the coupling element may be ellipsoidal, in the form of a disc or have other shapes depending on the geometry and other excitation requirements of the unit. It may also be noted that the annealing and ordering temperatures set forth in the body of the specification are for one particular substance having a specific composition; these temperatures must be altered for other materials and compositions in accordance with known criteria to produce the same results. Accordingly, from the foregoing remarks, it is understood that the present invention is to

be limited only by the spirit and scope of the appended claims.

What is claimed is:

1. A method for reducing the ferromagnetic resonance line width of an element of lithium ferrite material comprising:

grinding and polishing the element with fine abrasive grit;

applying material containing available lithium to the entire outer surface of said element; and

annealing the element while it is in contact with the applied material.

2. A method for treating an element of ferrite material having a volatile component comprising:

polishing the element with fine abrasive grit;

coating the ferrite material with a solution containing said volatile component; and

annealing the ferrite material while it is covered with the solution.

3. A method for treating an element of microwave material having a volatile component comprising:

polishing the element with fine abrasive grit;

contacting the entire surface of said element with an excess of said volatile component;

annealing the element while it is in contact with the excess of said component; and

ordering the material of said element at a temperature below the annealing temperature.

4. A method for treating an element of lithium ferrite comprising:

polishing the element with fine abrasive grit;

contacting the entire outer surface of said element with an excess of lithium;

annealing the element while it is in contact with the lithium; and

ordering the lithium ferrite element at a temperature below the annealing temperature.

5. A method for making a microwave element for use in the kilomegacycle frequency range comprising:

grinding and polishing an element of lithium ferrite having a chemical composition between  $Li_{0.1}Fe_{2.95}O_4$

and  $Li_{1.5}Fe_{2.2}O_4$ ;

applying a liquid containing available lithium to the element;

annealing said element at a temperature between 720°

C. and 900° C.; and

maintaining the lithium ferrite at a temperature near 700° C. to order the material.

6. A method for making a microwave element for use in the kilomegacycle frequency range comprising:

grinding and polishing an element of lithium ferrite having a chemical composition  $Li_{0.1}Fe_{2.95}O_4$  and  $Li_{1.5}Fe_{2.2}O_4$ ;

applying a liquid containing available lithium to the element; and

annealing said element at a temperature between 720° C. and 900° C.

#### References Cited by the Examiner

##### UNITED STATES PATENTS

|           |        |              |       |          |
|-----------|--------|--------------|-------|----------|
| 2,886,530 | 5/1959 | Greger       | ----- | 252—62.5 |
| 2,920,292 | 1/1960 | Scovil       | ----- | 333—24   |
| 2,922,125 | 1/1960 | Suhl         | ----- | 333—24   |
| 3,038,860 | 6/1962 | Vinal et al. | ----- | 252—62.5 |
| 3,093,588 | 6/1963 | Brown        | ----- | 252—62.5 |

##### FOREIGN PATENTS

|           |        |            |
|-----------|--------|------------|
| 167,179   | 4/1954 | Australia. |
| 1,242,007 | 8/1960 | France.    |

##### OTHER REFERENCES

IRE Transactions on Microwave Theory and Techniques, May 1961 (pages 272—273).

JOHN F. CAMPBELL, Primary Examiner.

HERMAN K. SAALBACH, Examiner.